

(No Model.)

3 Sheets—Sheet 1.

G. L. ROBERT.

PROCESS OF CONVERTING CRUDE IRON INTO MALLEABLE IRON OR STEEL.

No. 395,175.

Patented Dec. 25, 1888.

Fig. 1.



Fig. 2.



Fig. 3.



Fig. 4.



*Gustave L. Robert*

Inventor

*Witnesses*  
*John Hinkel Jr.*  
*John S. McMurtry*

*37 West 6th Street*

Attorneys

(No Model.)

3 Sheets—Sheet 2.

G. L. ROBERT.

PROCESS OF CONVERTING CRUDE IRON INTO MALLEABLE IRON OR STEEL.

No. 395,175.

Patented Dec. 25, 1888.

Fig. 5.



Fig. 7.



Witnesses

Prof. Hinkel, Jr.

H. S. McArthur

Gustav Louis Robert

Inventor

By J. T. & Son

Attorney

(No Model.)

3 Sheets—Sheet 3.

G. L. ROBERT.

PROCESS OF CONVERTING CRUDE IRON INTO MALLEABLE IRON OR STEEL.

No. 395,175.

Patented Dec. 25, 1888.

Fig. 5.



Fig. 6.



Fig. 7.



Witnesses  
John Hinkel Jr.  
Dr. S. McArthur

Gustave L. Robert  
Inventor  
By John H. Greenan

Attorney 5

# UNITED STATES PATENT OFFICE.

GUSTAVE L. ROBERT, OF STENAY, MEUSE, FRANCE, ASSIGNOR TO JOHN WESLEY BOOKWALTER, OF SPRINGFIELD, OHIO.

## PROCESS OF CONVERTING CRUDE IRON INTO MALLEABLE IRON OR STEEL.

SPECIFICATION forming part of Letters Patent No. 395,175, dated December 25, 1888.

Application filed November 14, 1888. Serial No. 290,776. (No specimens.) Patented in England May 9, 1888, No. 6,886.

*To all whom it may concern:*

Be it known that I, GUSTAVE LOUIS ROBERT, a citizen of the Republic of France, residing at Stenay, Department of the Meuse, Republic of France, have invented a new and useful Improvement in the Process of Converting Crude Iron into Malleable Iron or Steel, (for which I have obtained patent in England, No. 6,886, May 9, 1888,) of which the following is a full, clear, and exact specification.

In the conversion of crude or pig iron into malleable iron or steel by the use of air or oxidizing agent in an aeriform state for the purpose of oxidizing the combustible elements held in combination with the iron several fundamental conditions underlie and are essential to the perfection of the process, and to the extent to which they are co-ordinated in one general action depends the quality of the product. First, it is essential that the oxidizing agent shall come in contact with the iron and be distributed thereto in such manner and quantity, so intimately, and with such regularity as will secure the uniform oxidation of all the combustible elements held by the iron; secondly, it is important that the air shall come in contact with the metal in such manner that the eliminated impurities may not be caused to pass through the body of the metal to any material extent, and that when eliminated they shall remain as far as possible in a state of permanent separation from the metal; thirdly, it is of the greatest moment that the manner of bringing the air in contact with the iron shall be such that the elements of the iron shall be thoroughly oxidized while the air is as completely deoxidized as possible, in order that the smallest quantity consistent with rapid conversion and thorough combustion may be employed; fourthly, it is most desirable that a high temperature be maintained and the metal be brought to an extremely fluid condition without the use of any other fuel than that afforded by the combustible elements of the iron, and this is necessary in order to produce and maintain the highest possible temperature in the metal, which results in greater fluidity. Some of these requisites have long been known to those skilled in the art, and with the view of meeting them inventors have

heretofore, not unnaturally, adopted the practice of forcing the air through or into the interior of the body of metal, the general understanding of the requirements being that the intimate commingling of the air and the metal was of advantage in producing the required result. With this view they introduced the blast vertically through the bottom of the converter or horizontally into the body of the metal, or from above obliquely, but in all cases at a considerable depth below the normal surface of the metal, so as to penetrate the mass of metal in such manner that a portion of the metal throughout the operation of conversion was always above the air blast or current.

In order to more clearly explain the different effects which result from these different modes of applying the blast, I have appended diagrams in which I have attempted to indicate roughly what may be imagined to take place in a converter during such processes. The diagrams are all supposed to represent a vertical section of the metal in a converter, Figure 1 showing the blast introduced vertically at the bottom, Fig. 2 showing it introduced horizontally at or close to the bottom, and Fig. 3 showing it introduced at or near the top, but directed into the body of the metal.

In Fig. 1 the air is shown ascending through the whole body of the metal, causing violent ebullition and disturbance, everywhere throwing up the metal and impurities high above the surface, to which they fall back again, the arrows showing the return-currents bringing down the scoria to be again subjected to the pounding effects of the blast, and the impurities being driven into the body of the metal.

In Fig. 2 blasts are shown entering from opposite sides of the converter, and although these will not cause such violent disturbances as in Fig. 1, it will nevertheless be seen that the air permeates the greater part of the metal and that the return-currents from the surface drag down the scoria into the mass of the metal. This blast also being at a high pressure causes very violent disturbances of the whole mass, so that the scoria cannot remain quiescent at any one point.

In Fig. 3 the blast enters near the surface, and it is driven at once into the metal, with the result that violent agitation of the greater part

of the whole mass takes place and the scoria is formed in the metal, and after it rises to the surface it is again and again carried and forced down into the metal.

- 5 In all of these processes where the air enters and traverses the body of molten metal it is necessary to employ a powerful blast, using heavy and expensive machinery, and the air, after it has passed into the metal, tends 10 to force the particles of the latter apart and ascend to the surface in great bubbles, so that comparatively limited areas of metal are subjected to the action of the oxidizing agent, while the silicon, carbon, and other combustible elements are not brought into that intimate contact with the oxidizing agent which is essential to insure the most complete, rapid, and uniform combustion, and the force of the air-current and the great expansive action of 15 the air as it escapes from the surface of the bath produce both at the surface and in the body of the metal violent currents and vortices, while the descent of the metal thrown upward by the action of the blast increases the 20 agitation of the metal, so that the eliminated impurities are intimately mixed with and carried about in the bath by the powerful currents, and are returned again and again to the mouth of the tuyere and exposed to the pounding 25 effects of the blast and driven back into the body of the metal.

In consequence of the necessity of maintaining a high pressure of the blast in order to give the necessary penetrating effect into 30 and through the molten metal, the amount of oxygen supplied to the metal toward the completion of the conversion when most of the combustible elements have been removed is in excess of what is actually required, and the 35 utmost care is required to cut off the blast in such manner as to secure the desired converting effect without overoxidizing the iron.

A further objection incident to the above-specified modes of conversion results from the 40 fact that the highly-compressed air is richer in oxygen the instant when it enters the bath than during its subsequent progress, and naturally causes unequal oxidation, the oxidation being excessive and even destructive 45 near the mouth of the tuyere and deficient at or near the surface of the metal, where the air by expansion has resumed its natural volume, and as the point of rapid and greatest conversion is nearest the bottom of the bath, 50 and as the greatest amount of impurities are eliminated at this point, they must traverse the entire body of the metal before reaching the surface. This objectionable effect increases in degree as the combustible elements 55 of the iron are burned out, so that as the process of conversion approaches completion the danger of overoxidizing the iron greatly increases. It is not possible, therefore, by any of the 60 above-named processes to maintain that constant relation between the metal and the converting agent necessary to produce a uniform and determinate quality of metal, and the

process and the product are fitful and irregular.

It is the object of my invention to avoid the 70 unstable and involved conditions producing the variable, uncertain, and imperfect results heretofore specified and to establish conditions which are normally fixed, constant, and regular, while capable of being varied, adjusted, or modified, at the will of the operator, according to those variations in the conditions which result as the process of conversion is carried onward toward completion. In 75 effecting these results I take advantage of a well-known law of physics, that a violent atomic agitation of a liquid holding particles in suspension, or of a mixture of solid or semi-solid and fluid matters, will favor the separation of the mixed materials; but as such a violent agitation of the entire mass of metal in a converter at once would not be practicable, and as it would, moreover, be attended with the disadvantages before referred to of remixing the particles of impurities with 80 and among the particles from which they have been separated, and from which they should be maintained in a separated state, I depart from the methods heretofore employed of acting upon substantially the entire body 85 of metal at one time and subject limited portions only at a time to violent agitation and to the action of the oxidizing or converting agent, maintaining the greater portion in a comparatively quiet state, but bringing every 90 portion repeatedly within the area of violent agitation. It will therefore be evident that one of the primary characteristics of my process is that the body of molten metal is divided during the operation of converting 95 practically into two sections or portions in radically different conditions. One section is small in volume and the particles thereof are subjected to violent atomic action—that is, this portion is violently agitated and atomized or broken up into small particles—and as a result the impurities separate themselves from the metal, while the other portion, comprising the greater body, is comparatively 100 quiescent and free from violent commotions. 105

The greater violence of the action that is practicable to impart to limited portions of the metal results in a twofold effect. First, it favors rapid conversion, because such violent action separates and finely divides or atomizes the limited portions acted upon at one time, exposing large areas of surface to the converting agent; second, it secures the separation of the impurities by the natural action before referred to, whether these impurities 110 were in the crude metal or are formed in the bath during the process of conversion; and, third, it carries the particles of metal away from the area of violent agitation and conversion, so as to avoid continuous action of 115 the oxidizing agent on the same particles and brings in new metal to the agitating and converting area, thus preventing over-oxidation. 120

As one means of securing the desired

atomic disturbances of portions of the entire mass of molten metal, I make use of an oxidizing or converting blast, and I have found that this may be so directed upon the body 5 of metal as to violently agitate portions only of the same at one time, leaving the greater mass undisturbed except to the extent of imparting a desirable flow or gyration that repeatedly brings every portion into position to 10 be acted on directly by the blast.

In Fig. 4 of the accompanying diagram I have represented a vertical section of the converter and the bath with the blast introduced in a practically horizontal direction in a manner 15 to carry out my invention.

The blast is applied upon or so near to the normal surface of the metal in the bath and is so directed thereto that it will not enter or penetrate the body of the metal, as in former 20 processes, and so that practically no portion of the metal will be above the blast, and in such manner that but a small portion of the metal will be subjected to the action of the blast at any one time. Thus as the blast 25 passes inward in nearly a horizontal direction at a point adjacent to the surface of the metal its rapid forward motion, combined with the tendency to escape upward in the direction of least resistance, gives to the blast 30 and to the portion of metal carried therewith a resultant diagonally-upward direction away from the main body of metal, so that a small portion only of the metal is thus acted upon; but as this small portion is subjected to the 35 impact of the entire blast a much more violent agitation is imparted thereto by a comparatively light blast than it would be possible to impart to the entire body by a blast of the most powerful character, and as a result 40 of this agitation not only are the particles of impurities separated from the metal, but the latter is so spread or divided as to present the desired extended surfaces required to effect the speedy and thorough oxidation of 45 all particles. The action of the blast in carrying a portion of the metal to the opposite side of the converter is to pile up the metal at that side, which, together with the impact of the blast on the exterior portion of the 50 body of metal, results in the production of a circulatory or gyratory current in the direction of the arrows, which causes a flow of the metal downward and upward toward the area of violent action, while the metal is prevented 55 from rising above the line of the blast by the impact of the latter, which skins or beats off the particles presented in its path, so that an inclined surface is imparted to the bath at one edge lower and at the other higher than 60 the mouths of the tuyeres.

Inasmuch as the metal meets the air only at the surface of the bath there is no conversion below said surface and therefore the impurities formed are not carried through the 65 body of the metal as heretofore, but are skimmed from the surface thereof and thrown upward or to the other side of the converter,

and being once separated from the metal and of much less specific gravity they remain deposited upon the surface of the metal at that portion where the latter is in a comparatively quiescent condition, while the comparatively slow rate at which the body of the metal gyrates has not the effect in drawing down the eliminated particles below the surface. As 75 a result of the gradual elimination and collection of the impurities in a position separate from the metal, the body of the metal becomes gradually free from impurities and is subjected to the action of the blast again 80 and again in a constantly-purer condition, a radically different result from anything accomplished by processes of conversion heretofore employed in which there is no mechanical purification of the metal whatever, but on 85 the contrary the admixture of the impurities with the metal becomes greater as the process of conversion approaches completion. As an actual result of my improved process, the product is extremely free from impurities and 90 homogeneous in quality. As a result of the more perfect and rapid oxidation from the more thorough admixture of the atoms of air and metal, there is a higher temperature, inasmuch as there is a more complete and uniform conversion, and because, owing to the limited portion of metal acted upon at one time, every portion may be thoroughly oxidized. The temperature of the bath is therefore not only maintained as the result of the 100 action of the blast, but is increased so that the metal is rendered extremely fluid, thereby facilitating its movements under the action of the blast and preventing its rapid cooling when removed from the converter. 105

I have already referred to the danger of overoxidation in ordinary processes of the metal at the point where it comes in contact with the air at the mouth of the tuyeres because of its highly-compressed state and therefore increased richness in oxygen. It will be evident that this danger is averted by my process, since the compression of the air need be but very slight in order to drive away from the mouth of the tuyeres the small portion of metal which would tend to flow against the same if the tuyeres were placed at or slightly below the normal level of the metal in the converter. 115

From the foregoing it clearly appears that 120 the blast must not be too deep or it will enter into the body of the metal, while, on the other hand, it must be deep enough to come into sufficiently extensive and intimate contact with the metal to produce the necessary 125 reactions and conversion, or it will escape without producing the desired results; but it must be remembered that the bulk of the metal diminishes during the conversion by reason of the elimination of the impurities. 130 Consequently the level of the surface of the metal falls during the process and therefore the blast must be varied to maintain its position relatively to the metal. This may be

done in various ways, two of which naturally present themselves—first, by bringing the blast down to the metal, and, second, by bringing the metal up to the blast. The former proceeding may be most conveniently accomplished by using a tilting converter and turning it upon its trunnions, or, in a fixed converter, by having the tuyeres movable and dropping them as required. By thus adjusting the blast a continuous supply of new or fresh metal can be brought into the area or zone of conversion in such exact quantities as will maintain the proportion of the metal acted on relative to the volume of air as is necessary to the production of the best results. The raising of the level of the metal could be effected by adding more metal or by means of a false bottom, which would raise the whole of the metal or otherwise, so as by occupying part of the space previously occupied by the metal to restore the surface-level.

I will now describe apparatus which may be used in carrying out the foregoing process; but I wish it to be understood that I do not limit myself to the use of this apparatus, which forms the subject of an application for a patent filed by me August 30, 1887, Serial No. 248,578.

Figs. 5 and 6 show, respectively, a vertical section and a horizontal section, the latter through lines 1 2 3 4 of one of the arrangements, while Figs. 7 and 8 show in the same manner another arrangement of my converter. Fig. 9 is a sectional view of a tuyere. In Figs. 5 and 6 the converter, the cross-section of which is rectangular and has its corners rounded, receives a swinging motion on the journals A and A', supported by pedestals. This motion can be obtained by means of any mechanism such as that used for the manipulation of oscillating converters.

The tuyeres *a*, through which the blast is introduced, are arranged in a straight line, *x* *y*, on one side, *P*, only of the converter, and they open into a box or chamber, *C*, into which the blast enters through a supply-pipe, *T*. This box is provided with sliding glazed sight-holes *b*, preferably the same in number as there are tuyeres *a*, whereby the state of the tuyeres can be watched during the operation, and whereby, also, they can be cleaned or replaced with ease, and through which lime or other reagent can be inserted if required.

The side, *P*, chosen for the application of the tuyeres is preferably one presenting the greatest surface to the metal, and the plane in which the tuyeres are formed is parallel to the surface of metal and to the axis of rotation, A A', of the converter, so that whatever the inclination of the latter and the height of the metal in fusion may be the head of pressure on the orifices of all the tuyeres is equal. The cross-section of the tuyere-orifices is a rectangle having its corners rounded off, Fig. 9, thus injecting the blast in thin rectangular currents or sheets. This form gives with the same

sectional area a greater surface of contact between the air and the liquid metal.

In Figs. 7 and 8 the converter is of a substantially circular form in sectional plan, but with a straight face, *P*, parallel to the axis of rotation, A A', on which the tuyeres *a* are disposed, as before, on a horizontal line in plane parallel to the axis of the apparatus. The placing of all the tuyeres in one horizontal line parallel with the swinging axis enables the operator to maintain the proper relations between the tuyeres and the surface of the metal, and at any time to stop the operation almost instantaneously by simultaneously freeing all the tuyeres from the molten metal, this being done by turning the converter upon its trunnions.

The tuyeres placed thus horizontally form, with the straight face *P*, onto which they open, unequal angles, (see Fig. 8,) the magnitude of which varies with the form given to the cross-section of the apparatus. The object of this arrangement of the tuyeres is to facilitate the imparting of a gyratory motion to the metal in fusion, which motion exposes the molecules of metal successively to the oxidizing action of the blast at the surface of the fused metal.

By placing the tuyeres at different angles the horizontal rotary motion is prevented from becoming too violent, the impulse imparted by the blasts from the tuyeres having the greatest inclination being partially counteracted by those having less, these latter tending to blow the metal and scoria more directly across to the opposite side of the converter. By this means and the circumstance that all the tuyeres are in one horizontal line a comparatively feeble blast and an immersion of the tuyeres in the metal slightly below its nominal level are sufficient to oxidize the mass, and the reaction takes place at or near the surface.

The products of the reaction are therefore transmitted at once to the slag, instead of acting on the metal and the lining of the converter below.

I may subject successive limited portions of the entire bath to the action of the converting agent without imparting a gyratory motion to the body of metal, in which case other means of feeding it to the area of converting action must be employed.

I do not limit myself to the use of means described for securing the simultaneous conversion and violent local atomic agitation of the metal, nor to the specific construction of apparatus or arrangement of parts shown for carrying out said process, as this may be done with various means in different ways, as will be evident to those skilled in the art.

I do not herein claim the specific features described and claimed in my applications filed November 19, 1888, bearing Serial Nos. 291,189 and 291,190.

What I claim is—

1. The within-described improvement in converting crude iron into malleable iron or

steel, consisting in imparting to limited portions in succession of a bath of molten metal violent agitation in the presence of a converting agent, separating the impurities and the metal, returning the latter to the body of the metal in the bath and back from the body of metal in the bath to the area of agitation, and repeating these operations until all the metal has been acted on, the impurities are separated therefrom, and the conversion is complete, substantially as set forth.

2. The process of converting crude iron into malleable iron or steel, which consists in imparting to successive limited portions of a bath of molten metal a violent atomic agi-

tation and separating the metal and the impurities, returning the metal to the body of the bath and maintaining the eliminated impurities in their separated state, and repeating these operations until the entire body has been repeatedly operated upon, substantially as set forth.

In testimony whereof I have signed my name to this specification in the presence of two subscribing witnesses.

GUSTAVE L. ROBERT.

Witnesses:

F. L. FREEMAN,  
A. E. T. HANSMANN.